

Feb. 9, 1943.

D. A. EBERHARDT

2,310,356

ROLLING OF FLAT STRIPS

Filed Aug. 2, 1940



Inventor  
Daniel A. Eberhardt  
by John H. Cassidy  
His Attorney

## UNITED STATES PATENT OFFICE

2,310,356

## ROLLING OF FLAT STRIPS

Daniel A. Eberhardt, St. Louis, Mo.

Application August 2, 1940, Serial No. 349,409

4 Claims. (Cl. 80—60)

This invention relates to a method of forming flattened strips from a galvanized rod or wire.

An object of the invention is to provide a method of forming flat strips from galvanized rod or wire so as to avoid cracking the zinc coating. There are several advantages in the invention, one of which is economy. Galvanized rod or wire may be obtained commercially, and then rolled by the present process to produce a rust-proofed flat strip at a large saving, over the cost of first producing the flat steel shapes and then galvanizing those shapes. A second advantage is an improved product in its rust resisting characteristics, that is to say a flat strip prepared in accordance with this invention has been found to be superior in rust-resisting properties to strips which have been prepared by first rolling the steel and then galvanizing the strips. A third advantage is in the characteristics of the steel; that is in producing a steel which has a higher temper or a greater hardness than can be produced economically by ordinary hot dipped galvanizing. In the hot dip process of galvanizing, the temper of the steel and its hardness is reduced, while rolling by the present process raises the temper and increases the hardness.

Further advantages may be inherent in the process, and may be apparent from the following detailed description.

The drawing is an elevation showing apparatus which may be used in practicing the process in this invention.

The apparatus consists essentially of a pair of opposed rolls 1 and 2, which are driven simultaneously by a motor 3. The rolls have opposed surfaces, by which the blank may be shaped to form the flat strips. These surfaces may be such as to form two sides on the strips which are parallel, or the rolled surfaces may be such as to form other shapes.

As a rod or wire or blank B is fed to the rolls 1 and 2 it is wetted by a lubricant, such as turpentine. This wetting agent is contained in a trough 4, into which dips a wheel or grooved pulley 5 to elevate by capillary attraction a sufficient quantity of the lubricant to wet the blank B as it passes to the rolls. This wetting is facilitated by a bristle brush 6, as specifically shown in the drawing.

The rolls are driven by the motor 3 through speed reducing means so as to give a desired speed to the rolls. Thus, the motor 3 has on its shaft a pulley 7, driving a belt 8 which drives a pulley 9. The pulley 9 has on its shaft a small pulley 10 with a belt 11 connecting with a large

pulley 12 on the shaft of which is keyed a pinion 13, meshing with a gear 14 keyed to the shaft of the roll 2.

The rolls 1 and 2 are power connected by gears 15.

The wetting wheel 5 is driven by the gear 14 meshing with and driving a pinion 16 keyed to the shaft of the wheel 5.

Guide rollers 17 and 18 are positioned in front of the rolls 1 and 2, and rollers 19 and 20 in the rear of the rolls. Straightening rolls, not shown, both in front of and behind the pressure rolls may be employed.

It is known, of course, that it is common practice to roll flat metal shapes from round bar or stock, but it has heretofore been assumed that it was impossible to roll galvanized or zinc coated wire, because of the tendency of the coating to crack. In practicing the present invention, however, advantage has been taken of the peculiar properties of zinc, so that in rolling the zinc does not crack. Zinc when cold is brittle, is malleable at 120°-150° C. (250°-300° F.), and is very brittle at 200 C.

It has been found that by rolling the stock at a speed sufficient to heat the stock at the rolls by the action of the rolls to a temperature at which the zinc is malleable, satisfactory results are obtained. This temperature is, as indicated, between 250 and 300° F. It has been found that this temperature is readily obtainable and maintained when operating at room temperatures without the application of any heating or cooling medium by maintaining a proper speed. It is possible, of course, to supplement the heat obtained from the action of the rollers by applying heat or it is possible to cool the work in order to maintain the proper temperatures.

It has been found in practice that satisfactory results are obtained, provided the stock is not deformed beyond certain limits so that the elongation of the zinc coating does not substantially exceed 25% in any direction. Or, more particularly, the best results are obtained while deforming the stock in such a manner that the longitudinal elongation of the zinc coating is substantially uniform with its lateral elongation, and this longitudinal elongation should not be in excess of 25%. The longitudinal elongation with respect to the lateral elongation can be controlled by increasing or decreasing the size of the rollers. Other factors being equal, the larger the rolls the less longitudinal elongation will be secured and vice versa.

A difficulty or a problem presented by the roll-

ing of the galvanized stock at the temperature indicated, has been overcome or solved by the use of a wetting agent or lubricant. If the galvanized stock is passed through the rolls at the temperature indicated while dry, particles of the zinc coating will adhere to the rolls, and will soon cause difficulty. This is avoided by wetting this stock with a proper agent as it is about to be placed between the rolls. Many satisfactory wetting agents or lubricants have been found, among them some are turpentine, kerosine, gasoline and vinegar. Such a wetting agent should be such as not to oxidize or discolor or spot the surface; it should be volatile, so that it will be expelled from the article by the heat imparted by rolling to avoid the necessity of cleaning the strips. It should also be safe so as to avoid damage of fire or injury to the operator. Of the wetting agents, which have been mentioned, turpentine has been found to fulfill the requirements. It is cheap enough for economical use; it presents no hazards; it evaporates completely from the strips without any special attention; it operates sufficiently as a lubricant; and it does not oxidize, discolor or spot the product. It is not doubted, however, that other wetting agents quite as satisfactory may be found and utilized.

By way of example to illustrate the invention, and not by way of limitation, a typical operation may be described. The stock selected is 10-gage soft galvanized merchants or fence wire, which is well known commercially. This stock has a temper equivalent to that of No. 4 or No. 5 cold rolled steel. This wire is passed between 5" rolls after it has been wetted with turpentine. The rolls are so formed as to produce a flat cross section approximately  $\frac{1}{8}'' \times \frac{1}{8}''$ , and the rolls are driven at a speed to pass the stock at the rate of approximately 240 ft. per minute.

It has been found that this operation produces a satisfactory product with a longitudinal elongation of approximately 20%. The lateral elongation of the surface coating is approximately the same. The size of the rolls and the speed of pass must, of course, be different for stock and shapes of different sizes. It has been found that the surface coating of zinc is not damaged by

the process, but if anything its efficacy as a rust preventing agency is increased. At any rate, the product in this respect is superior to that obtained commercially by galvanizing preformed strips and the hardness and temper of the stock is materially increased.

While the blank was of soft steel, the finished product has a hardness approximately equal to No. 1 cold rolled steel. A typical piece tested 10 showed a Rockwell hardness of B-95.

Various changes may be made in the details of operation within the scope of the appended claims, parts of the invention may be used without the whole, and various improvements and 15 steps may be added thereto.

I claim:

1. The method of forming flattened strips comprising passing a galvanized rod between pressure rolls at a pressure sufficient to substantially deform the rod and at a speed sufficient to heat the rod at the rolls by the action of the rolls from room temperature to a temperature between 250° and 300° F.

2. The method of forming flattened strips comprising passing a galvanized rod between pressure rolls at a pressure sufficient to substantially deform the rod while maintaining a temperature between 250° and 300° F. in the rod at the rolls.

3. The method of forming flattened strips comprising passing galvanized rod having a zinc coating between pressure rolls at a pressure sufficient to substantially deform the rod while maintaining such a temperature in the rod at the rolls at which the zinc is malleable and will not crack under the deformation caused by the rolls.

4. The method of forming flattened strips comprising passing a galvanized rod having a zinc coating between pressure rolls at a pressure sufficient to substantially deform the rod while maintaining a temperature in the rod at the rolls at which the zinc is malleable and will not crack under the deformation caused by the rolls, and while limiting the change in form of the rod so that the elongation of the zinc coating does not substantially exceed 25% in any direction.

DANIEL A. EBERHARDT.